

1

3,095,374

## LUBRICATING COMPOSITION

Richard E. Baus, Philadelphia, and Earl E. Fisher, Glenolden, Pa., assignors to Gulf Oil Corporation, Pittsburgh, Pa., a corporation of Pennsylvania  
No Drawing. Filed Apr. 25, 1957, Ser. No. 655,003  
4 Claims. (Cl. 252—18)

This invention relates to lubricating compositions and their preparation and particularly to lubricating compositions having wear and corrosion-reducing characteristics which suit them for use in the lubrication of internal combustion engines.

Due to the conditions encountered in the lubrication of the cylinders of internal combustion engines, particularly the formation of acids, the wear of piston rings, cylinders and cylinder walls is frequently excessive. Petroleum lubricating oils in general need improvement to combat excessive wear which occurs under engine operating conditions.

While the problem of combatting engine wear is important in the lubrication of all types of internal combustion engines, the problem is particularly serious in the lubrication of low-speed marine diesel engines which operate on fuels having high sulfur content. It is known, for example, that residual fuel oils can be used to power low-speed marine diesel engines in lieu of the more costly lighter diesel fuels. However, as is well known, heavier petroleum fractions generally contain higher concentrations of sulfur than do the lighter fractions. Experience has shown that diesel engines operating on these heavy high sulfur fuels have serious maintenance problems in the form of excessive cylinder wear. It is believed that the high concentration of sulfur in the fuel is responsible in great part for the excessive wear since fuel containing large quantities of sulfur can cause both corrosion and erosion of cylinder walls and pistons. The corrosive wear occurring within engines operating on this type of fuel has been attributed specifically to the acidic vapors such as sulfur dioxide and sulfur trioxide formed on combustion of the sulfur containing fuels. In the presence of water which is formed during combustion and which may result from moist air entering the engine through the air intake, these sulfurous vapors attack the exposed metal parts.

It has now been found that improved liquid lubricating compositions which exhibit excellent antivear properties are provided by a uniform blend of a major amount of a lubricating oil and a minor amount sufficient to confer improved wear properties to the composition of magnesium carbonate and a small amount of a magnesium stearate sufficient to maintain the magnesium carbonate uniformly suspended in the lubricating oil.

The lubricating oil which constitutes the major ingredient of the new composition is selected from a wide variety of lubricating oils such as naphthenic base, paraffinic base and mixed base mineral oils. In general, any mineral oil of lubricating viscosity or synthetic lubricating oils such as polymerized olefins, organic esters such as di-2-ethylhexyl sebacate and azelate and the like, are used as the base oil to form a lubricating composition in accordance with this invention. For the lubrication of low speed marine diesel engines a mineral lubricating oil having a viscosity in the range 1000 to 3000 Saybolt seconds at 100° F. is generally employed.

The magnesium carbonate is dispersed and maintained suspended uniformly throughout the lubricating oil base to impart to the composition the desired wear and corrosion-reducing characteristics. By having the magnesium carbonate present in the lubricating oil in this

2

manner, it is available as a protective coating on the metal surfaces of the cylinder to effectively neutralize the acidic combustion products thus preventing metal surfaces from attack. The magnesium carbonate is employed as a finely divided powder in order to assist in obtaining stable suspensions. In general, the size of the magnesium carbonate particles should be on the order of 20 microns or less, preferably 2 microns.

As has been stated, a sufficient amount of magnesium carbonate is employed to confer improved wear properties to the resulting lubricating composition. The specific amounts to employ vary with the severity of the lubricating services required. For example, using fuel containing little sulfur and with the engine in substantially continuous service, as little as 0.1% by weight of magnesium carbonate in the total composition is sufficient. However, with high sulfur fuels and/or intermittent engine service, larger amounts are required and amounts of magnesium carbonate as high as 10% by weight or higher can advantageously be employed. For many applications including the cylinder lubrication of low speed marine diesel engines burning high sulfur fuels, 3% by weight of magnesium carbonate is satisfactory and is preferred.

The magnesium stearate additive of the invention is either a neutral magnesium stearate, that is, magnesium distearate, or a basic magnesium stearate, that is, magnesium hydroxy stearate wherein only one hydroxyl group has been neutralized with the stearic acid. Both of these materials as well as mixtures thereof are substantially equally effective for the purposes of this invention.

Although both the magnesium stearate and magnesium carbonate coact in the compositions of the invention to reduce corrosion and wear within the cylinder, the magnesium stearate additive functions primarily as a dispersing and suspending agent to maintain the magnesium carbonate effectively and uniformly dispersed throughout the lubricating oil base. While stable lubricating compositions are obtained when the magnesium stearate is employed in amounts as small as 0.25% by weight of the composition, the maximum amount of magnesium stearate should not exceed about 6% to avoid gelation of the composition to form a grease. Where the magnesium stearate is employed in amounts of from about 0.25% to about 6% by weight, the magnesium carbonate is maintained in proper and permanent distribution throughout the lubricating oil base and does not tend to separate readily therefrom, the entire composition nevertheless being a liquid as desired and not a grease. In a preferred composition, 1 percent by weight of magnesium stearate is employed.

The improved lubricating compositions of the invention are prepared by mixing the magnesium carbonate and the magnesium stearate, in amounts sufficient to give a desired concentration in the final composition, with a portion, as for example one half, of the base lubricating oil. This mixture is then heated with continuous agitation to a temperature of from 250° to 350° F. or higher, to dissolve the magnesium stearate. When the magnesium stearate has been completely dissolved, the remaining portion of the base lubricating oil is added while maintaining a temperature of 250° to 350° F. The mixture is then cooled with continuous agitation to a temperature of about 100° F. or lower. Using this procedure gel formation is effectively prevented and a uniformly blended, stable, liquid lubricating oil composition is obtained.

The following examples further illustrate the invention, which is not to be construed as limited thereby. In these examples, the base oil employed was a blended lubricating

oil obtained from mixtures of dewaxed, solvent refined lubricating oil stocks, having the following inspection.

|                      |      |
|----------------------|------|
| Gravity, ° API       | 25.1 |
| Viscosity, SUV, sec. | 1050 |
| 100° F.              | 5    |
| 210° F.              | 80.1 |

|                  |     |
|------------------|-----|
| Flash, O.C., ° F | 475 |
| Fire, O.C., ° F  | 530 |

#### EXAMPLE I

10

A stable, anti-wear lubricant composition is prepared by adding magnesium carbonate and magnesium hydroxy stearate in the amounts indicated below to a portion constituting approximately 50% of the oil base. The resulting slurry is heated to approximately 300° F. while being constantly agitated. When the magnesium hydroxy stearate has been completely dissolved, and while maintaining the temperature at approximately 300° F., the remaining portion of the oil base is added. The composition is then cooled to 100° F. with continued agitation. The final 15 lubricating oil composition had the following make-up and inspection.

|                             |      |
|-----------------------------|------|
| Make-up, percent by weight: |      |
| Oil base                    | 96.0 |
| Magnesium carbonate         | 3.0  |
| Magnesium hydroxy stearate  | 1    |

|                                                                         |      |
|-------------------------------------------------------------------------|------|
| Inspection:                                                             |      |
| Gravity, ° API                                                          | 22.2 |
| Viscosity, SUV, sec.:                                                   | 30   |
| 100° F.                                                                 | 1987 |
| 210° F.                                                                 | 236  |
| Flash, O.C., ° F                                                        | 495  |
| Fire, O.C., ° F                                                         | 545  |
| Neutralization value, ASTM D 664-54 (potentiometric): Total base number | 35   |
| 2.20                                                                    |      |

#### EXAMPLE II

Utilizing the same procedure as in Example I, a composition is prepared having the following make-up and 40 inspection.

|                             |      |
|-----------------------------|------|
| Make-up, percent by weight: |      |
| Oil base                    | 95.0 |
| Magnesium carbonate         | 3.0  |
| Magnesium hydroxy stearate  | 2.0  |

45

|                                                                         |      |
|-------------------------------------------------------------------------|------|
| Inspection:                                                             |      |
| Gravity, ° API                                                          | 21.8 |
| Viscosity, SUV, sec.:                                                   | 3160 |
| 100° F.                                                                 | 1325 |
| 210° F.                                                                 | 50   |
| Flash, O.C., ° F                                                        | 495  |
| Fire, O.C., ° F                                                         | 545  |
| Neutralization value, ASTM D 664-54 (potentiometric): Total base number | 4.70 |

#### EXAMPLE III

55

Utilizing the same procedure as in Example I, a composition is prepared having the following make-up.

|                             |    |
|-----------------------------|----|
| Make-up, percent by weight: |    |
| Oil base                    | 96 |
| Magnesium carbonate         | 3  |
| Magnesium stearate          | 1  |

#### EXAMPLE IV

60

Utilizing the same procedure as in Example I, a composition is prepared having the following make-up.

|                             |    |
|-----------------------------|----|
| Make-up, percent by weight: |    |
| Oil base                    | 93 |
| Magnesium carbonate         | 3  |
| Magnesium stearate          | 4  |

#### EXAMPLE V

65

Utilizing the test described above, a comparison of the antiwear properties of the lubricating oil composi-

lubricating oil base and in the one instance 0.1% by weight of magnesium carbonate and 0.25% by weight of magnesium stearate, and in the other instance 10% by weight of magnesium carbonate and 6% by weight of magnesium stearate.

The stability of the lubricating compositions containing the magnesium additives is determined by subjecting a measured volume of the composition to varying temperatures over a 48 hour period. Inspection of the sample is made at various temperatures and the percent separation by volume determined. Using this procedure the following results were obtained:

|                                      | Oil of Ex. I | Oil of Ex. II | Oil of Ex. III | Oil of Ex. IV |
|--------------------------------------|--------------|---------------|----------------|---------------|
| Stability test, separation, percent: |              |               |                |               |
| 24 hours:                            |              |               |                |               |
| 0° F.:                               |              |               |                |               |
| Oil                                  | Nil          | Nil           | Nil            | Nil           |
| Sediment                             | Nil          | Nil           | Nil            | Nil           |
| 32° F.:                              |              |               |                |               |
| Oil                                  | Nil          | Nil           | Nil            | Nil           |
| Sediment                             | Nil          | Nil           | Nil            | Nil           |
| Ambient temperature:                 |              |               |                |               |
| Oil                                  | Nil          | Nil           | Nil            | Nil           |
| Sediment                             | Nil          | Nil           | Nil            | Nil           |
| 130° F.:                             |              |               |                |               |
| Oil                                  | Nil          | Nil           | Nil            | Nil           |
| Sediment                             | Nil          | Nil           | Nil            | Nil           |
| 150° F.:                             |              |               |                |               |
| Oil                                  | Nil          | Nil           | Nil            | Nil           |
| Sediment                             | Nil          | Nil           | Nil            | Nil           |
| 180° F.:                             |              |               |                |               |
| Oil                                  | 0.5          | Nil           | 1              | Trace         |
| Sediment                             | Nil          | Nil           | Nil            | Nil           |
| 48 hours:                            |              |               |                |               |
| 0° F.:                               |              |               |                |               |
| Oil                                  | Nil          | Nil           | Nil            | Nil           |
| Sediment                             | Nil          | Nil           | Nil            | Nil           |
| 32° F.:                              |              |               |                |               |
| Oil                                  | Nil          | Nil           | Nil            | Nil           |
| Sediment                             | Nil          | Nil           | Nil            | Nil           |
| Ambient temperature:                 |              |               |                |               |
| Oil                                  | Nil          | Nil           | Nil            | Nil           |
| Sediment                             | Nil          | Nil           | Nil            | Nil           |
| 130° F.:                             |              |               |                |               |
| Oil                                  | Nil          | Nil           | Nil            | Trace         |
| Sediment                             | Nil          | Nil           | Nil            | Nil           |
| 150° F.:                             |              |               |                |               |
| Oil                                  | Trace        | Nil           | Nil            | Nil           |
| Sediment                             | Nil          | Nil           | Nil            | Nil           |
| 180° F.:                             |              |               |                |               |
| Oil                                  | 1            | Trace         | 3              | 1             |
| Sediment                             | Nil          | Nil           | Nil            | 1             |

As seen from the above data, there is very little tendency for the magnesium additives to separate from the oil base even at temperatures not normally encountered in storage. Accordingly, the wear reducing and corrosion inhibiting properties imparted to the lubricating compositions of the invention by the magnesium compounds are effectively maintained while permitting the composition to be stored for extended periods.

To illustrate the wear reducing properties of the improved lubricating compositions of this invention a four ball wear test is conducted as follows: Three steel balls are securely fastened so that rotation is impossible. A fourth steel ball in a rotating spindle is placed so that it is entirely supported by the other three balls forming a pyramid. The three immobile steel balls and the rotating single steel ball are forced into contact with each other in response to a vertically applied load. Sufficient test lubricant is poured into a test cup to cover the three lower balls at a predetermined depth. The spindle is revolved at 1800 r.p.m. while electrical heating units heat the oil to a temperature of 266° F. At the conclusion of the test, wear is measured by examination of the scars on the clean surfaces of the three stationary balls; the two maximum right angle diameters of each wear scar being measured to the closest 0.01 mm. and averaged. The antiwear properties are rated by the difference in the scar diameters. The actual pressure exerted on each point of contact is calculated as a function of the lever load and the scar diameter.

Utilizing the test described above, a comparison of the antiwear properties of the lubricating oil composi-

tions containing the magnesium additives with the base oil is shown in Table II.

Table II

|                                 | Base oil | Oil of Ex. I | Oil of Ex. II |    |
|---------------------------------|----------|--------------|---------------|----|
| Test conditions:                |          |              |               |    |
| Spindle speed, r.p.m.           | 1,800    | 1,800        | 1,800         |    |
| Level load, kg.                 | 7.5      | 7.5          | 7.5           | 10 |
| Duration of test, hr.           | 1        | 1            | 1             |    |
| Temperature of test:            |          |              |               |    |
| ° C.                            | 130      | 130          | 130           |    |
| ° F.                            | 266      | 266          | 266           |    |
| Oil temperature rise, ° C.      | 0        | 0            | 0             |    |
| Average coefficient of friction | 0.112    | 0.0967       | 0.0928        |    |
| Average scar diameter, mm.      | 0.57     | 0.38         | 0.28          |    |
| Mean specific pressure, p.s.i.  | 17,100   | 38,880       | 73,470        | 15 |

As seen from the above results, the lubricating compositions of the invention reduce wear from 33% to 50% and more as compared with the base oil containing no additives.

The ability of the lubricating compositions of this invention to effectively neutralize the acidic products formed upon combustion suits these compositions particularly for the lubrication of large low speed marine diesel engines which operate on high sulfur content fuels, such as residual oils and distillates which contain free or combined sulfur in amounts anywhere from 0.1% to 6% and more by weight. The lubricating compositions of this invention are suited for this type of lubrication also because of the nature and quantity of the ash produced when the lubricants are burned. As is known, separate cylinder lubrication is employed in large marine diesel engines and the lubricant is subjected to combustion within the cylinder. The magnesium additives of this invention produce upon combustion an ash of a light and fluffy nature which is easily blown from the cylinder of the engine without the formation of harmful deposits therein.

It is to be noted that while the lubricating oil compositions of the invention are particularly suited for the lubrication of marine diesel engines which operate on high sulfur content fuel, the utility of the new compositions is not limited thereto. As seen from the results of the wear test reported in Table II, the new lubricants possess excellent wear reducing characteristics independent of their acid neutralizing properties. Thus, the new compositions may be advantageously utilized in the lubrication of all types of internal combustion engines.

In addition to the additives disclosed herein, there may be present in the lubricating compositions of this invention other conventional additives such as pour point depressants, anti-rust agents, oiliness improvers, extreme pressure agents, viscosity index improvers and the like.

The present invention provides liquid lubricating compositions which are remarkably effective for reducing wear and corrosion of the cylinders of internal combustion engines. The new compositions possess additional

characteristics which particularly suit them for use in the lubrication of marine diesel engines which operate on high sulfur contents fuels. A further advantage of the lubricating compositions of the invention is that the compositions possess a high degree of stability which permit them to be stored for extended periods of time without having their effectiveness to reduce wear and corrosion in cylinders lost or materially diminished.

The expression "consisting essentially of" as used in the claims means that the lubricating composition is made up of the components recited and these components are the characterizing ones. But the expression does not exclude the presence of minor amounts of materials which do not materially affect the basic and novel characteristics of the composition:

Resort may be had to the various modifications and variations which fall within the spirit of the invention and the scope of the appended claims.

We claim:

1. A stable liquid lubricating composition consisting essentially of a uniform blend of a mineral lubricating oil containing from about 0.1% to 10% by weight magnesium carbonate and from 0.25% to 6% by weight of a magnesium stearate.
2. A stable liquid lubricating composition consisting essentially of a uniform blend of a mineral lubricating oil containing about 3% by weight magnesium carbonate and about 1% by weight of a magnesium stearate.
3. A process for preparing a uniformly blended stable liquid lubricating composition which comprises adding to a portion of a lubricating oil, magnesium carbonate and a magnesium stearate, the magnesium carbonate being added in an amount sufficient to constitute from .1% to 10% by weight of the final composition, the magnesium stearate being added in an amount sufficient to constitute from .25% to 6% by weight of the final composition, heating the mixture with continuous agitation to dissolve the said magnesium stearate, adding additional lubricating oil in an amount sufficient to form a final composition of desired concentration, then cooling the said mixture with continuous agitation to obtain a uniformly blended liquid anti-wear lubricating composition.
4. The process of claim 3 wherein the said mixture is heated to a temperature of about 250° to 350° F.

#### References Cited in the file of this patent

#### UNITED STATES PATENTS

- |    |           |                        |               |
|----|-----------|------------------------|---------------|
| 50 | 2,079,051 | Sullivan et al. -----  | May 4, 1937   |
|    | 2,417,431 | McLennan -----         | Mar. 18, 1947 |
|    | 2,485,861 | Campbell et al. -----  | Oct. 25, 1949 |
|    | 2,671,758 | Vinograd et al. -----  | Mar. 9, 1954  |
| 55 | 2,676,925 | Lindstrom et al. ----- | Apr. 27, 1954 |
|    | 2,781,314 | Wassen -----           | Feb. 12, 1957 |
|    | 2,832,677 | Morway et al. -----    | Apr. 29, 1958 |

#### FOREIGN PATENTS

- |    |         |                     |              |
|----|---------|---------------------|--------------|
| 60 | 200,149 | Australia -----     | Nov. 4, 1955 |
|    | 716,648 | Great Britain ----- | Oct. 13 1954 |

UNITED STATES PATENT OFFICE  
CERTIFICATE OF CORRECTION

Patent No. 3,095,374

June 25, 1963

Richard E. Baus et al.

It is hereby certified that error appears in the above numbered patent requiring correction and that the said Letters Patent should read as corrected below.

Column 1, line 22, for "lubricaiton" read -- lubrication --; line 69, for "characeristics" read -- characteristics --; column 2, line 38, for "carbontae" read -- carbonate --; column 4, in the table, the last nine lines thereof should appear as shown below instead of as in the patent:

|          |       |       |     |       |
|----------|-------|-------|-----|-------|
| 130° F.: |       |       |     |       |
| Oil      | Nil   | Nil   | Nil | Trace |
| Sediment | Nil   | Nil   | Nil | Nil   |
| 150° F.: |       |       |     |       |
| Oil      | Trace | Nil   | Nil | 1     |
| Sediment | Nil   | Nil   | Nil | Nil   |
| 180° F.: |       |       |     |       |
| Oil      | 1     | Trace | 3   | 1     |
| Sediment | Nil   | Nil   | Nil | Nil   |

column 5, lines 46 and 47, for "independend" read -- independent --.

Signed and sealed this 31st day of December 1963.

(SEAL)

Attest:

ERNEST W. SWIDER

Attesting Officer

EDWIN L. REYNOLDS

Acting Commissioner of  
Patents